

## UNITED STATES PATENT OFFICE

1,930,178

COMPOSITION FOR PRINTING OR  
GRAINING

Logan A. Mizener, Wilmette, Ill., assignor to  
Chicago Mill and Lumber Corporation, Chi-  
cago, Ill., a corporation of Delaware

No Drawing. Application January 26, 1931  
Serial No 511,434

9 Claims. (Cl. 134—28)

This invention relates to the art of printing and more particularly to the art of printing or graining certain types of wood to simulate other woods having distinctive appearing grains. A particular object of the invention is to provide a composition and process by which hard or soft, plain textured woods which are relatively inexpensive and plentiful may be printed upon, or grained so as to simulate more costly varieties of wood which are in demand because of their definite and characteristic grain. Another object of the invention is to provide a printing ink or composition for the purpose described having qualities of durability and ease of application, and which will quickly set and immediately resist smearing or rubbing off after being applied to the surface for which it is intended. A still further object of the present invention is to provide a printing compound and process for use in printing or marking on either a wet or dry base which may be wood or other materials but which has particular adaptability in printing upon a wet base. Still another object of the invention is to provide a composition for the purpose described which will be simple and inexpensive to prepare and compound, efficient in use and which may be prepared and used by unskilled workmen to produce effective results.

Other and further objects of the invention will be apparent from the disclosure in the following specification.

This invention has particular adaptability in the cigar box industry in which wood such as so-called Spanish cedar which has a distinctive aroma and grain has been used extensively for packing good grades of cigars and tobacco. The tobacco purchasing public has thus through a period of years come to the point of associating the aroma and particularly the grain of Spanish cedar with high grade tobacco. A demand has thus been created by producers of tobacco products for wooden containers which, by their appearance, will produce the impression that high grade tobacco is packed therein.

As Spanish cedar and similar wood is becoming increasingly scarce and less accessible, there is a desire on the part of manufacturers of tobacco products to utilize less expensive woods and yet retain substantially all the sales advantages of the more expensive wood. One manner of accomplishing this result has been to glue extremely thin veneer of Spanish cedar or mahogany to plain textured, inexpensive woods which are more plentiful than are Spanish cedar or mahogany at the present time. Paper has also been printed

to imitate the grain of the wood and containers of ordinary plain wood have been covered therewith.

Another suggested method has been to print or grain the surface of this less expensive plain textured wood with marks or lines so as to simulate the grain of the more desirable varieties. However, many difficulties have been encountered in printing directly on the wood itself, because heretofore it has never been deemed practicable to print on wood until after it has been dried to about the normal moisture content of kiln dry wood. The reason for this has been that the graining compounds in use could not give satisfactory results unless the lumber or wood were dried down to a certain low point of moisture content. If the lumber had an excess of moisture the ink would run and blur and the narrow lines which are most needed to simulate grain could not be readily obtained because the ink would spread and smear and instead of lines there would be more or less blurry markings. It has also been found that the surface of the wood to be treated becomes hard and dense when the moisture is removed, and, in knife-cut lumber particularly, portions of the surface having a softer texture and greater moisture absorption capacity collapse in the drying process more than the portions of lesser absorption capacity regardless of how mechanically true and perfect the surface may have been when cut from the wet or green logs or fletches. Because of this harder character after drying much wear and tear is caused to the printing machinery, especially to the impression means such as printing rolls or the like. In addition, it is difficult and nearly impossible to obtain a uniform application of the graining ink to dry, unfinished lumber because of the irregularities of the surface arising during the drying; and even when the board has been surfaced there yet remains a certain amount of warp or twist, as well as considerable rigidity, in the lumber, which causes damage to the machinery involved in the printing operation. For these reasons the production of printed lumber or boards has always been a more or less slow, uncertain and cumbersome operation, and the cost has therefore been too great to warrant production on a substantial scale.

When the printing composition of the present invention is used the particular amount of moisture contained in the impression receiving base is not material even when this moisture content reaches its upper levels. This finds particular application in the case of the utilization of rotary

cut lumber or so-called veneer stock due to the fact that the logs are always impregnated with considerable moisture before going to the lathe or other device on which the lumber is cut. This moisture content may vary considerably depending upon whether a given piece of lumber has been cut from the log near its outer surface or near the center. It has been found that the weight of the sap wood, that is, the wood adjacent to the outside of the log, with the moisture therein, is frequently 75% to 100% greater than the bone dry weight of this portion of the log but this percentage may decrease considerably toward the center. For example, one species of gum has been found to vary from 118% moisture in the sap wood to 82% moisture near the heart for a sixteen inch diameter log which has been immersed for several hours in a bath of hot water. The compound of the present invention finds particularly advantageous use, compared with printing compounds heretofore known, in operating on freshly cut, so-called veneer lumber having a moisture content in excess of 20%. The present invention, however, is not confined in its use to wet lumber but gives very desirable results on lumber of ordinary commercial dryness and kiln dried lumber. By the terms "wet wood" or "wet lumber" as used herein any lumber having a moisture content in excess of that present in air dry lumber is to be understood. The present compound is applicable to lumber in any of its forms, although it is usually applied to thinner cut boards which may be produced either by sawing, slicing or rotary cutting.

In preparing the printing compound, it is desirable to employ a carrying vehicle such, for example, as a starchy substance which may be prepared with water to assume a thick consistency as by means of cooking. Corn starch is very well adapted for the purpose since it is comparatively inexpensive and easily available and is simple to prepare for the present purpose. Any other starch such as potato or tapioca flour or the like can be used.

To the desired amount of starch in an aqueous medium any desired coloring matter may be added. Aniline colors have been found very satisfactory in this respect, being simple to handle and giving desirable results.

To this mixture of starch and coloring matter is added a quantity of glycerine and vinegar, the last mentioned ingredient being preferably cider vinegar having approximately a 4% acetic acid content. Any other suitable acetic acid containing substance may be employed for this purpose. It is of particular note in this connection that apparently the interaction between the glycerine and acetic acid is an important factor in giving to the compound its good adhering properties, particularly when applied to wet lumber, since these ingredients combine to form a water resistant compound which serves to retain the ink upon the wood fibers regardless of the moisture that may be present in the wood.

It has been found in practice, where lumber fresh from the cutter or slicer is grained, that the temperature of the lumber will govern to a great extent the desirable proportion of glycerine to acetic acid. In the usual method of preparing logs for slicing or rotary cutting, they are first subjected to the ordinary steaming process or to a water bath which is controlled to maintain a temperature ranging from in the neighborhood of 165° to about 200° F., more or

less. The steaming process or water bath renders the wood soft and water-soaked to a degree varying with the texture or density of the particular variety of wood subjected to a given length of treatment. This facilitates cutting the sheets or slabs of lumber from the log or flitch with a minimum of tearing of the fibrous structure. Lumber treated in this way still retains a temperature of about 150° F., more or less, upon leaving the lathe or slicer, the temperature varying according to the cooling effects of the prevailing atmospheric conditions.

In carrying out the process it has been found that when the temperature of the wet material operated upon is at about ordinary room temperature fairly good results can be obtained where the glycerine content of the compound is present in the proportion of about one part of glycerine to about eight parts vinegar. However, if the lumber is to be treated fairly soon after leaving the cutter and while having a temperature considerably above ordinary room temperature, it has been discovered that more dependable results are obtained with a glycerine content of about one part of glycerine to six or seven parts of vinegar; but if the conditions are such that it is desirable to grain the lumber almost immediately after leaving the cutter and before it has had time to cool, and especially during warm weather, a higher glycerine content should be used to avoid spreading or "whiskering" of the grain or other design. In fact, when graining warm wood direct from the cutter, a quantity of glycerine in about the proportion of one to four parts vinegar has been found very satisfactory. It is apparent, therefore, that a glycerine content within a range of one in about four to eight parts vinegar will prove suitable under a variety of particular conditions. However, I do not wish to be limited to these exact proportions since it has been determined that the glycerine content may be somewhat varied above and below the proportions given depending upon various factors such as moisture and temperature. It may be noted, however, that when the glycerine content is raised much above one part to four parts of vinegar the composition is likely to become gummy and sticky and has a tendency to smear when applied.

When the ingredients mentioned have been mixed together, it has been found desirable to cook the mass until it has reached a suitable thickness or viscosity. After the composition has cooled, preferably to about atmospheric temperature, it is ready for use.

The following example will illustrate a preferred form of the present embodiment of the invention:

|                                  | Parts by weight |
|----------------------------------|-----------------|
| Starch                           | about 96        |
| Coloring matter (aniline colors) | about 15        |
| Glycerine                        | about 8-16      |
| Cider vinegar (4% acetic acid)   | about 64        |
| Water                            | about 450       |

A graining compound or ink prepared as above described and in the proportions given has proved very effective in practice and particularly when woods of softer texture are grained, either dry or wet.

In the above example the starch may be varied between 90 and 100 parts with relation to the rest of the mixture or in certain cases other suitable fillers may replace part of the starch. The amount of vinegar may be varied between 60 and 150

70 parts. The amount of coloring matter used depends more or less upon the intensity of the particular dyes employed and the intensity of the results that are desired. Water soluble aniline 5 colors have been found very desirable in carrying out the present invention. Generally speaking, the amount of color may be varied within very wide limits depending upon what particular type of coloring matter is used as well as the effect desired to be obtained. The variation of the glycerine and vinegar with relation to each other has previously been discussed in some detail. The amount of water may be varied within certain limits depending upon the purity and moisture content of the other ingredients. For example, if pure acetic acid is employed then more water will be necessary, but if a vinegar having an acetic acid content of less than about 4% is used and consequently more of this ingredient 10 is necessary, then a proportionally smaller amount of water will be needed. Atmospheric conditions also affect the amount of water required. In any event, the amount of water should be such as to give the mass a jelly-like 15 consistency after it has been prepared by cooking as above stated and allowed to cool.

After it has been prepared by cooking as above stated, the mixture is preferably allowed to stand in a comparatively large vessel so that it will 30 cool slowly. This tends to cure the mass and gives it the proper consistency for efficient application. The preferred time for cooling has generally been found to be about 15 hours where the ink is applied by the roller type of printing mechanism.

It is apparent from the foregoing that the composition may be varied within certain limits to be effective under a varying range of conditions both of the moisture and temperature of the lumber and the general conditions and temperature of the atmosphere. The composition is one that can be readily made up without requiring a 40 large amount of skill on the part of the operative.

While the composition of the above described 45 formula gives entirely satisfactory results for moderate speeds and when the lumber is of substantially uniform and comparatively soft texture, nevertheless it has been found that where a considerable range of extreme conditions is 50 present in the lumber or other impression receiving material the inclusion of additional ingredients, with the composition heretofore described, insures obtaining satisfactory results under these extreme conditions. This is true where any one 55 or more of a combination of conditions prevail, for example, where the atmosphere is warm and humid and the lumber comes to the printing mechanism at a temperature not much reduced from the temperature at which it leaves the severing mechanism, or the wood is of comparatively 60 hard texture or the printing mechanism is running at a comparatively high speed with the wood of relatively high moisture content. To this end it has been developed that if certain albuminous substances such, for example, as blood 65 albumin in its various forms or other proteids or albumins are mixed with the above described product and properly controlled so as to time the setting qualities of the resulting composition at 70 the proper point of application of the ink, it is rendered still more efficient and certain without danger of blurring or "whiskering" in spite of relatively high temperatures and speeds, or moisture content of the material operated upon.

71 Furthermore, by the addition of such albuminous

substances the setting of the ink is accelerated and the color tone and durability of the finish are improved.

It is a well-known fact that blood albumin has the property of coagulating and forming a water-insoluble substance when subjected to heat. It is also a known fact that certain chemicals such as paraformaldehyde will act upon blood albumin in a cold liquid medium to cause it to congeal and set, without the application of heat, to form a fairly water-resistant compound.

While paraformaldehyde is capable of reacting with the blood albumin to cause it to coagulate and form a tough, water resistant coating, it has been found necessary to employ an alkaline substance which will retard the action of the paraformaldehyde as long as the mixture is maintained in relatively large masses and which will lose its effect upon the paraformaldehyde, either by evaporation or by combination, when the composition has been applied as a relatively thin film upon the surface being imprinted. Ammonium hydroxide has been found well suited for this purpose.

In preparing a preferred form of the albuminous addition to the composition, a desired quantity of light or dark blood albumin is soaked in a liquid medium until it can be stirred to an even consistency. Thereupon the retarding agent and coagulant are stirred into the albumin mixture. The addition of a small amount of salt is often desirable in the composition as a preservative, particularly where the climate is such that there is danger of the organic matter putrifying on account of its standing for some time prior to use. 100 However, the salt is most beneficial when aniline colors are employed because it enhances both the brightness and setting of the colors. The use of this latter ingredient is optional, of course, and may be omitted without deleterious effects if 110 desired.

The blood albumin portion is preferably made up of the following ingredients in about the following proportions by weight:

|                                        | Parts    |
|----------------------------------------|----------|
| Blood albumin (light or dark) _____    | about 30 |
| Ammonium hydroxide (Sp. G. 0.90) _____ | about 1½ |
| Paraformaldehyde _____                 | about 4½ |
| Water _____                            | about 37 |
| Sodium chloride _____                  | about 8  |

The amounts of ammonium hydroxide and paraformaldehyde may be varied between 1 and 2 parts and 4 and 5 parts respectively. As has been previously brought out, the blood albumin containing composition will, due to the coagulant, set without the application of heat; however, since the wet lumber is generally put through some sort of heated dryer to expedite removal of the excess moisture, there will, as a rule, be a further setting action upon the blood albumin by reason of the heat. Heat is not, however, essential to form a satisfactory grained surface.

The blood albumin portion of the printing composition is separately prepared and then added by agitation to a batch of the color carrying compound which may be made up as previously outlined. The resultant mixture takes on a jelly-like form when fully prepared and may be kept for many hours prior to use by keeping the exposed surface of the mass damp as by laying dampened cloth thereon.

After numerous experiments and tests I have concluded that the various reactions taking place in the compound as a result of adding the albumin

composition may be described as follows. The two batches of ingredients, after being prepared separately, are mixed together after the first mixture described herein has been allowed to cool and become properly cured. The first batch retains substantially the acid characteristics imparted to it by the acetic acid and color and the albumin batch retains the alkalinity characteristic of its components. On mixing the two batches together there is no doubt a reaction initiated between the acetic acid and the ammonium hydroxide but this interaction is apparently retarded to a large extent by the viscosity of the agglomerate due largely to the starch. In any event, it appears that sufficient alkalinity is retained in those parts of the mixture containing the paraformaldehyde so as to leave sufficient ammonium hydroxide to effectively retard or inhibit any action by the paraformaldehyde on the blood albumin for eighteen or more hours after the two batches have been mixed together. However, when the prepared ink is spread in a thin film on the impression receiving base, which is generally somewhat acid, the ammonium hydroxide is dissipated, either due to the acidity of the base or because the additional moisture with which the film comes in contact on the impression receiving surface enables a more intimate contact of this alkaline substance and the acid of the composition; or the ammonia which is volatile may be almost instantly evaporated because of the thinness of the film and the heat of the base. Nevertheless, upon application of the ink there appears to be an immediate action of the paraformaldehyde upon the blood albumin to set it and, together with the other ingredients causing the formation of a clear, permanent impression of the desired design.

A graining composition produced in accordance with the present disclosure lends itself admirably to rapid quantity production of artificially grained lumber to simulate Spanish cedar, mahogany or the like. This composition may also be used to reproduce advertising designs or wording upon wooden panels used for various purposes such as shipping cases or boxes and the like in a similar manner to that described for the graining operation. The desired design, whether a grain, advertising matter or other markings, may be printed or impressed upon the receiving surface by means of impression mechanism of any suitable character and having suitable impression means such as the recessed cylindrical printing roll or other more or less conventional means. In operation this impression applying mechanism may be operated as close to the point at which the lumber is cut from the log as is practical; and the graining may be carried on as rapidly as it is physically possible to handle the output. The ink sets so rapidly after application that there is no staining of the superimposed unprinted surface of the lumber as it is stacked in coming off the press prior to removal to the dryer.

It has been found in practice that the use of lumber having a considerable moisture content when applying the graining composition of the present invention has many advantages. Outstanding among these advantages is the fact that the surface presented to the printing rolls or other impression means is as true and smooth as when the material leaves the cutting mechanism because the plane of the surface has not been varied by reason of collapsing of the less dense portions of the wood which ordinarily occurs

as a result of drying, as has been heretofore explained. Furthermore, since the wood fibers are more resilient and pliable due to their water-soaked condition, the wet lumber will cause a minimum of wear and tear to the printing rolls or machinery. Another great advantage of this process lies in the fact that one drying operation suffices both for drying out the veneer as well as for completing the drying and setting of the graining ink.

Excellent results have been obtained by using such plain woods as red gum, tupelo, cottonwood, magnolia, black gum, poplar, basswood and lynn for the base upon which to apply the graining effect. However, there are other woods which may be used with equally favorable results.

While the invention is particularly applicable to printing on wood it is not to be considered as entirely limited thereto as it can be applied to advantage for printing on other substances, especially when they have a moisture content substantially above normal.

While the present description sets forth a preferred embodiment of the invention, numerous changes may be made in the process and compound without departing from the spirit of the invention, and it is, therefore, desired that the present embodiment be considered in all respects as illustrative and not restrictive, reference being had to the appended claims rather than to the foregoing description to indicate the scope of the invention.

I claim:

1. A printing compound adapted for application to wet lumber comprising a suitable starch and water mixture to provide a pasty base, mixed together with water-soluble aniline color, glycerine and vinegar, the starch, glycerine and vinegar being present in the mixture in approximately the following quantities:

|           | Parts by weight | 115 |
|-----------|-----------------|-----|
| Starch    | 90 to 100       |     |
| Glycerine | 8 to 16         |     |
| Vinegar   | 60 to 70        | 120 |

2. A composition adapted for use in simulating the grain of desirable woods which comprises starch, glycerine, coloring matter, acetic acid, blood albumin, ammonium hydroxide and paraformaldehyde.

3. A graining composition comprising in one part starch, glycerine and acetic acid and comprising in another part blood albumin, ammonium hydroxide and paraformaldehyde, said parts being separately prepared and said second mentioned part being commingled in said composition by agitation.

4. A graining composition comprising in one part a relatively cool mixture of starch, glycerine, coloring matter and acetic acid, and comprising in another part blood albumin, salt, ammonium hydroxide and paraformaldehyde, said parts being separately prepared and said last mentioned part being commingled in said composition by agitation.

5. A composition or ink adapted for application to freshly cut wet lumber to form distinctive markings thereon and comprising in one part starch, coloring matter, glycerine, vinegar and water brought to a thick consistency by cooking and then cooling, and another part comprising blood albumin, said parts being commingled by agitation.

6. A composition of matter comprising in combination by weight approximately 90 to 100 parts

80

85

90

95

100

105

110

115

120

125

130

135

140

145

150

starch, 8 to 16 parts glycerine, 60 to 70 parts vinegar, 30 parts blood albumin, 1 to 2 parts ammonium hydroxide, and 4 to 5 parts paraformaldehyde.

- 5 7. A composition adapted for printing upon a hot impression receiving base of considerable moisture content and somewhat acidic reaction, consisting of two commingled parts, one part comprising pigment carried in a thick mass of cooked starch, acetic acid and glycerine, and a second part comprising blood albumin, paraformaldehyde as a congealing agent for said blood albumin and ammonium hydroxide as a retarding agent to substantially prevent action of said congealing agent on said blood albumin while the same are in a mass, said ammonium hydroxide becoming dissipated upon application of the composition to the impression receiving base whereupon the paraformaldehyde immediately acts upon the albumin to congeal it and form a water-resistant compound.
- 10 8. A composition for printing on a wet base comprising coloring matter, a water resistant compound comprising a mixture of vinegar and glycerine, an additional water resistant com-

pound comprising blood albumin and sufficient paraformaldehyde to congeal the blood albumin, and a quantity of ammonium hydroxide sufficient to inhibit the action of the paraformaldehyde for a substantial length of time, all of said ingredients being mixed and intermingled with a starchy base of jelly-like consistency whereby dissipation of the volatile portions of the ammonium hydroxide will be retarded until a film of the compound is deposited on the wet base.

15 9. In a printing composition, a water resistant compound comprising a mixture of vinegar and glycerine, an additional water resistant compound comprising blood albumin and sufficient paraformaldehyde to congeal the blood albumin, and a quantity of ammonium hydroxide sufficient to inhibit the action of the paraformaldehyde for a substantial length of time, all of said ingredients being mixed and intermingled with a starchy base of jelly-like consistency whereby the dissipation of the volatile portions of the ammonium hydroxide will be retarded for any unexposed aggregate of the mixture until said aggregate has been exposed to the atmosphere.

LOGAN A. MIZENER. 100

30  
35  
40  
45  
50  
55  
60  
65  
70  
75

105  
110  
115  
120  
125  
130  
135  
140  
145  
150